

1

3,829,290

**REACTION OF SODIUM CELLULOSATE WITH MONO- AND DIFUNCTIONAL EPOXIDES IN NON-AQUEOUS MEDIA**

Ralph J. Berni, Metairie, Ruth R. Benerito, New Orleans, and Donald M. Soignet, Metairie, La., assignors to the United States of America as represented by the Secretary of Agriculture

No Drawing. Filed June 29, 1972, Ser. No. 267,313

Int. Cl. D06m 13/10; C08b 11/08

U.S. Cl. 8—120

16 Claims 10

**ABSTRACT OF THE DISCLOSURE**

Fibrous cellulose ethers have been prepared by a non-aqueous process comprising preparing a sodium cellulose with suitable Cellulose I content in preparation for reaction with an epoxide to yield a derivative generally useful in the field of permanent press textiles.

A non-exclusive, irrevocable, royalty-free license in the invention herein described, throughout the world for all purposes of the United States Government, with the power to grant sublicenses for such purposes, is hereby granted to the Government of the United States of America.

This invention relates to the chemical treatment of cellulosic textiles. Specifically, this invention relates to the chemical treatment of cellulosic textiles in non-aqueous media to yield cellulosic derivatives in the form of textiles which are useful in the permanent press field. More specifically this invention relates to the preparation of a cellulose fabric which contains a suitable quantity of sodium ion to be quickly thereafter reacted with a certain epoxide.

The primary object of this invention is to provide a process for reacting mono- and diepoxides with cotton cellulose.

Another object of this invention is to provide a process which attaches sodium ions to the cellulose structure at the hydroxyls so that in combination with the swelling caused by the same reagent prepares the Cellulose I lattice for reaction with epoxides thus producing a series of new ether derivatives of cellulose.

A third object of this invention is to provide new cellulosic ethers which find utility in the preparation of permanent-press textiles.

**Definition:** The word "sodacell" as employed throughout this specification has reference to a specific form of cellulose which contains specific quantities of sodium ions ( $Na^+$ ) in a swollen cellulose structure which contains the Cellulose I lattice.

In the prior art sodacell has been disclosed by Berni et al. in a paper bearing the title "Anion-Exchange Cottons Prepared From Sodium Cellulose" which appeared in Textile Research Journal, vol. 40, pp. 999-1006 (1970). Sodacell has been used recently as a substrate for the chemical modification of cotton in nonaqueous media. In early work, fashioned after methods described by Schwenker and Pascu, and later others, sodacell fabrics were prepared by reaction of sodium methoxide with cotton in methanol. Later research recognized the advantages of using premercerized fabric converted to Group IA metal cellulosates for further chemical modification.

Projections of this work which disclose the details of the present invention can be found in a paper by Berni et al., bearing the title "Sodium Cellulosate and Diethylaminoethylcellulose as Substrates for Modification of Cotton With Epoxides." At this writing such paper is "In Press" in Industrial and Engineering Chemistry—Product Development.

Earlier studies made use of aqueous base pretreatments of cotton prior to its reaction with epoxides in various solvents.

2

Now we have discovered that certain sodium celluloses prepared by reacting methanolic solutions of sodium methoxide with solvent exchanged cottons and other cellulosic materials will provide the suitable form of Cellulose I lattice in the cotton or other textile to cause the reaction of these derivatives with certain epoxides.

Many difunctional epoxides were reacted in concentrations of from 0.28 to 1.70 moles/liter of solution in tertiary butanol or in perchloroethylene in the process of investigation. The degree of substitution (D.S.) accomplished ranged from about .01 to .08. Most of the investigative work was carried out using cotton fabric to provide suitable material for textile testing.

In general the present invention can best be described as a process for preparing fibrous cellulose ethers which yield textile products, many of which are suitable for permanent-press garments and other household goods, the steps of the process comprising:

(a) Preparing a sodium cellulose with Cellulose I lattice containing about from 0.1 to 3 milliequivalents of sodium ion per gram of cellulose,

(b) Immediately thereafter reacting the sodium cellulose of step (a) with an epoxide selected from the group consisting of:

allylglycidyl ether,  
butadiene diepoxide,  
butadiene monoepoxide,  
diglycidyl ether of 1,4-butanediol,  
diglycidyl ether of glycerol,  
diglycidyl ether of ethyleneglycol,  
epichlorohydrin,  
glycidyl methacrylate,  
octadiene diepoxide,  
phenyl glycidyl ether, and  
vinylcyclohexene diepoxide

in organic solvent selected from the group consisting of:  
perchloroethylene, and  
tertiary butanol

for about from 3 to 17 hours, at about from 25° to 105° C., using the lower temperatures with the longer periods of time, to produce a fibrous cellulosic ether derivative having a degree of substitution of about from .01 to .08.

By the process of the present invention reaction of mono- and diepoxides with cotton cellulose and/or cellulose derivatives such as viscose rayon, ramie, dialdehyde cotton, partially acetylated cotton, and carboxymethylated cotton can be carried out by subjecting the selected material to treatment with a swelling agent and reacting with sodium methoxide in methanol in order to attach  $Na^+$  to the cellulosic hydroxyls. While the sodium cellulose of the selected cellulosic material is still deprived of oxygen and all contact with water then it is reacted with the selected epoxide. Resiliency and/or increased elongation is developed in the fibers so that a fabric prepared by the process of this invention is substantially wrinkle free when compressed and released in the dry and/or in the wet state.

There is, however, an alternate step to the process of this invention. That step includes the strengthening of the fiber by a pretreatment with 23% sodium hydroxide and solvent exchanging the water out prior to step (a) of the process.

Resilience, as viewed here, is the ability to recover from deformation and particularly as it applies to a quality or the property of fabrics. Whether or not a given chemically treated cellulosic material exhibits this property can best be evaluated by one of the several available physical tests commonly employed in textile testing laboratories. The Monsanto Wrinkle Recovery Test was chosen here. This particular test measures the crease angle

of fabrics, as a criterion for evaluation of resiliency imparted to the treated fabrics. This test is fully described in the text of American Society for Testing Materials Designation D1295-60T.

Those skilled in the art feel that the "conditioned wrinkle recovery angle" should be at least 250° (warp plus filling) before it can be said to be resiliant to the lowest acceptable degree.

Prior art processes for the treatment of cellulose with mono- and diepoxides employ cellulose pretreated with aqueous sodium hydroxide and with immediate immersion into carbontetrachloride solutions of only one epoxide, butadiene diepoxide, giving a product with increase wet and dry resiliency. Prior art processes require good solubility of the epoxide employed in aqueous basic solution. This seriously limits the scope of the epoxides that can be employed. The process of the present invention can utilize any number of non-aqueous solvents, including primarily t-butanol or perchloroethylene, which are excellent solvents for innumerable epoxides. The use of these solvents allows finishing either completely or partially free from water systems which add to pollution problems. Solvent finishing with this type process can be accomplished with almost complete recovery of solvent used.

#### APPLICABLE EQUATIONS

##### (1) Preparation of the sodium celluloseate:



##### (2) Reaction of the sodacell with an epoxide:

(a)



(b)



5 bleached, was placed in a reaction tube equipped with an inlet and an outlet for liquids and gases. About 300 ml. of dry dimethylformamide (DMF) was added to the vessel and the fabric was allowed to swell for 16 hours. The DMF solution was then allowed to drain, and dry methanol was added and drained three times to remove DMF and final traces of water.

10 A methanolic solution (300 ml.) of sodium methoxide (ca. 1 molar) was added to the vessel and the fabric was allowed to react for 75 minutes while dry nitrogen was bubbled through the chamber. The sodium methoxide solution was drained and three 300 ml. additions of t-butanol were used to remove excess sodium methoxide and solvent. The t-butanol and the fabric could be allowed to stand under dry nitrogen for indefinite periods before re-action, if necessary.

15 Using the preferred method, the fabric was removed from the chamber, a small test sample was removed for titration of Na<sup>+</sup> content, and then the sodacell was placed in a graduated cylinder (250 ml. used) containing 30 grams of the diglycidyl ether of glycerol dissolved in t-butanol which had been preheated in an oven for 1 hour at 70° C. The graduated cylinder containing the reaction mixture was then placed back in the oven for 4 hours.

20 The fabric was then removed, neutralized with 5% acetic acid solution, rinsed 3 times in methanol, and washed for 30 minutes in 60° C. tap water to remove all unreacted materials. The fabric was then ironed dry, allowed to equilibrate for 4 hours and weighed. The fabric had a weight add-on of 14.3%. The original sodacell had a Na<sup>+</sup> content of 1.06 meq./g. of fabric. The fabric had a conditioned (dry) and wet wrinkle recovery of 25 271° and 264°, respectively (warp and fill). The fabric maintained 60% of its original breaking strength and essentially all of 6.3% elongation at break.

#### EXAMPLE 2

30 The following examples are shown to illustrate that butadiene diepoxide and epichlorohydrin significantly improve dry wrinkle recovery and that other epoxides, although they etherify cotton, do not significantly improve dry wrinkle recovery to above permanent press minimum acceptable levels at these add-ons. Fabrics were treated as in Example 1 with exceptions as noted in the table.

| Epoxide (30 g./250 ml.) <sup>1</sup> | Na <sup>+</sup> , meq./g. <sup>2</sup> | Add-on, percent | Wrinkle recovery (W+F) degrees | Breaking strength, Dry, lbs. | Elong. at break, percent |
|--------------------------------------|----------------------------------------|-----------------|--------------------------------|------------------------------|--------------------------|
| Butadiene diepoxide                  | 1.05                                   | 18.2            | 234                            | 233                          | 22.5                     |
| Epichlorohydrin                      | 1.04                                   | 4.9             | 255                            | 222                          | 18.1                     |
| Butadiene monoepoxide                | 1.16                                   | 2.3             | 196                            | 174                          | 35.9                     |
| Allyl glycidyl ether                 | 1.07                                   | 4.9             | 186                            | 178                          | 27.1                     |
| Vinylcyclohexene diepoxide           | 1.11                                   | 1.7             | 205                            | 192                          | 30.6                     |
| Diglycidyl ether of 1,4-butanediol   | 1.00                                   | 8.9             | 240                            | 209                          | 8.7                      |
| Phenyl glycidyl ether                | 1.05                                   | 8.2             | 204                            | 180                          | 33.9                     |
| Glycidyl methacrylate                | 1.05                                   | 7.1             | 223                            | 177                          | 28.6                     |
| Control                              |                                        |                 | 189                            | 176                          | 45.6                     |
|                                      |                                        |                 |                                |                              | 6.9                      |

<sup>1</sup> Epoxide dissolved in 250 ml. (total volume) of t-butanol at 70° C. and reacted for 4 hrs.

<sup>2</sup> Milliequivalents of sodium ion per gram of fabric.

70 The following examples are provided to illustrate the invention and should not be construed as limiting the invention in any manner whatever.

#### EXAMPLE 1

A sample of 80 x 80 cotton printcloth weighing approximately 10 grams, which had been desized, scoured, and

75 bleached, was placed in a reaction tube equipped with an inlet and an outlet for liquids and gases. The following examples are shown to illustrate that the diglycidyl ether of glycerol is the preferred epoxide to significantly improve dry and wrinkle recovery when perchloroethylene is used as solvent in place of t-butanol as in Example 1. Other epoxides used etherified cotton but did not increase wet or dry wrinkle recovery to mini-

imize permanent press levels at these add-on levels as shown in the following table:

| Epoxide (30 g./250 ml.) <sup>1</sup> | Na <sup>+</sup> ,<br>meq./g. <sup>2</sup> | Add-on,<br>percent | Wrinkle<br>recovery<br>(W+F)<br>degrees |     | Breaking<br>strength<br>(lbs.) | Elong. at<br>break<br>(percent) |
|--------------------------------------|-------------------------------------------|--------------------|-----------------------------------------|-----|--------------------------------|---------------------------------|
|                                      |                                           |                    | Dry                                     | Wet |                                |                                 |
| Diglycidyl ether of glycerol         | 0.70                                      | 26.7               | 274                                     | 265 | 32.7                           | 6.2                             |
| Butadiene diepoxyde                  | 0.71                                      | 19.4               | 239                                     | 195 | 26.9                           | 4.0                             |
| Epichlorohydrin                      | 0.67                                      | 4.6                | 243                                     | 211 | 24.8                           | 6.3                             |
| Diglycidyl ether of 1,4-butanediol   | 0.76                                      | 12.8               | 243                                     | 198 | 31.2                           | 7.2                             |
| Octadiene diepoxyde                  | 0.72                                      | 5.9                | 219                                     | 208 | 28.7                           | 6.7                             |

<sup>1</sup> Epoxide (30 g.) dissolved in perchloroethylene (250 ml. total volume) at 70° C. Fabrics were reacted for 3 hours.

<sup>2</sup> Milliequivalents of sodium ion per gram of fabric.

#### EXAMPLE 4

The following examples are shown to illustrate that high wet wrinkle recovery could be obtained with the epoxides when 23% NaOH is used as swelling solvent with the use of 5 solvent exchanges of methanol to remove final traces of water, and 0.6 M NaOCH<sub>3</sub> for preparation of sodacell as in Example 1 with some exceptions listed in the following table:

| Epoxide (30 g./250 ml.) <sup>1</sup> | Na <sup>+</sup> ,<br>meq./g. <sup>2</sup> | Add-on,<br>percent | Wrinkle<br>recovery<br>(W+F)<br>degrees |     | Breaking<br>strength<br>(lbs.) | Elong. at<br>break<br>(percent) |
|--------------------------------------|-------------------------------------------|--------------------|-----------------------------------------|-----|--------------------------------|---------------------------------|
|                                      |                                           |                    | Dry                                     | Wet |                                |                                 |
| Diglycidyl ether of glycerol         | 1.53                                      | 40.0               | 231                                     | 290 | 30.8                           | 19.7                            |
| Butadiene diepoxyde                  | 1.76                                      | 38.8               | 256                                     | 265 | 18.3                           | 14.1                            |
| Epichlorohydrin                      | 1.54                                      | 8.8                | 228                                     | 267 | 18.0                           | 20.4                            |
| Vinyl cyclohexene diepoxyde          | 1.44                                      | 6.0                | 165                                     | 267 | 41.0                           | 27.3                            |
| Diglycidyl ether of 1,4-butanediol   | 1.41                                      | 18.0               | 197                                     | 309 | 25.2                           | 22.7                            |
| Glycidyl methacrylate                | 1.39                                      | 15.0               | 174                                     | 260 | 41.3                           | 26.8                            |
| Phenyl glycidyl ether                | 1.57                                      | 15.7               | 179                                     | 224 | 47.2                           | 25.8                            |
| Allyl glycidyl ether                 | 1.47                                      | 11.7               | 135                                     | 198 | 42.8                           | 31.2                            |
| Butadiene monoepoxide                | 1.48                                      | 7.0                | 161                                     | 247 | 49.3                           | 29.3                            |
| Control (untreated)                  |                                           |                    | 189                                     | 176 | 45.6                           | 6.9                             |
| Control (23% NaOH)                   |                                           |                    | 184                                     | 206 | 57.3                           | 28.7                            |

<sup>1</sup> Epoxide dissolved in 250 ml. (total volume) of t-butanol at 70° C. and reacted for 4 hours.

<sup>2</sup> Milliequivalents of sodium ion per gram of fabric.

#### EXAMPLE 5

Fabrics treated as in Example 4 with the exception that 45 perchloroethylene was used as solvent for the epoxides used and the reaction time and temperature varied as shown in the following table:

(b) immediately thereafter reacting the sodium cellulose of step (a) with an epoxide selected from the group consisting of:  
allylglycidyl ether,  
butadiene diepoxyde,  
butadiene monoepoxide,  
diglycidyl ether of 1,4-butanediol,  
diglycidyl ether of glycerol,

| Epoxide compound                    | Weight<br>(grams) <sup>1</sup> | Na <sup>+</sup> ,<br>meq./g. <sup>2</sup> | Reaction<br>conditions |                  | Wrinkle recovery<br>(W+F) <sup>o</sup> |     | Breaking<br>strength,<br>(lbs.) | Elong.<br>at break<br>(percent) |
|-------------------------------------|--------------------------------|-------------------------------------------|------------------------|------------------|----------------------------------------|-----|---------------------------------|---------------------------------|
|                                     |                                |                                           | Time<br>(hr.)          | Temp.,<br>(° C.) | Add-on,<br>percent                     | Dry |                                 |                                 |
| Diglycidyl ether of glycerol        | 30                             | 1.11                                      | 3                      | 70               | 41.9                                   | 232 | 265                             | 32.4                            |
|                                     | 10                             | 1.40                                      | 0.5                    | 105              | 9.7                                    | 219 | 253                             | 36.0                            |
|                                     | 20                             | 1.40                                      | 0.5                    | 105              | 11.7                                   | 233 | 227                             | 34.9                            |
|                                     | 30                             | 1.40                                      | 0.5                    | 105              | 11.8                                   | 255 | 244                             | 38.6                            |
|                                     | 30                             | 1.40                                      | 17.0                   | 30               | 12.5                                   | 198 | 219                             | 39.6                            |
| Epichlorohydrin                     | 30                             | 1.21                                      | 3                      | 70               | 9.5                                    | 214 | 267                             | 27.1                            |
| Diglycidyl ether of 1,4-butanediol  | 30                             | 1.22                                      | 3                      | 70               | 27.0                                   | 220 | 249                             | 34.1                            |
|                                     | 10                             | 1.40                                      | 0.5                    | 105              | 5.9                                    | 196 | 206                             | 38.7                            |
|                                     | 20                             | 1.40                                      | 0.5                    | 105              | 7.9                                    | 235 | 195                             | 38.1                            |
|                                     | 30                             | 1.40                                      | 0.5                    | 105              | 8.8                                    | 221 | 210                             | 40.5                            |
| Diglycidyl ether of ethylene glycol | 30                             | 1.40                                      | 0.5                    | 105              | 13.3                                   | 236 | 206                             | 30.6                            |
| Octadiene diepoxyde                 | 30                             | 1.19                                      | 3.0                    | 70               | 14.3                                   | 205 | 292                             | 24.5                            |
| Control                             |                                |                                           |                        |                  |                                        | 189 | 176                             | 47.4                            |

<sup>1</sup> Grams of epoxide in 250 ml. of perchloroethylene solution.

<sup>2</sup> Milliequivalents of sodium ion per gram of fabric.

We claim:

1. A process for preparing under anhydrous conditions 70 fibrous cellulose ethers which yield textile products, the process comprising:

(a) preparing a sodium cellulose with Cellulose I lattice containing about from 0.1 to 3 milliequivalents of sodium ion per gram of cellulose by reacting a cel- 75

vinylcyclohexene diepoxyde dissolved in an organic solvent selected from the group consisting of perchloroethylene and tertiary butanol for a period of about from 3 to 17 hours, at about from 25° to 105° C., using the lower temperatures with the longer periods of time, to produce

- a fibrous cellulosic ether derivative having a degree of substitution of about from .01 to .08.
2. The process of Claim 1 wherein the epoxide is allyl-glycidyl ether.
3. The process of Claim 1 wherein the epoxide is butadiene diepoxide.
4. The process of Claim 1 wherein the epoxide is butadiene monoepoxide.
5. The process of Claim 1 wherein the epoxide is di-glycidyl ether of 1,4-butanediol.
6. The process of Claim 1 wherein the epoxide is di-glycidyl ether of glycerol.
7. The process of Claim 1 wherein the epoxide is di-glycidyl ether of ethylene glycol.
8. The process of Claim 1 wherein the epoxide is epichlorohydrin.
9. The process of Claim 1 wherein the epoxide is glycidyl methacrylate.
10. The process of Claim 1 wherein the epoxide is octadiene diepoxide.
11. The process of Claim 1 wherein the epoxide is phenyl glycidyl ether.
12. The process of Claim 1 wherein the epoxide is vinylcyclohexene diepoxide.
13. The process of Claim 1 wherein the solvent is per- 25 chloroethylene.

14. The process of Claim 1 wherein the solvent is tertiary butanol.
15. The allylglycidyl ether of cellulose prepared by the process of Claim 1.
16. The butadiene ether of cellulose prepared by the process of Claim 1.

## References Cited

## UNITED STATES PATENTS

- 10 3,293,073 12/1966 Goodman et al. ----- 8—120 X  
3,372,977 3/1968 Berni et al. ----- 8—120

## OTHER REFERENCES

- Berni et al.: article in Textile Research Journal, vol. 15 40, No. 11, November 1970, pp. 999—1006.
- McKelvey et al.: article in Textile Research Journal, vol. 29, 1959, pp. 918—925.
- Avney et al.: article in Textile Research Journal, vol. 38, 1968, pp. 599—605.
- HERBERT B. GUYNN, Primary Examiner  
U.S. Cl. X.R.  
260—231 A